

## UNITED STATES PATENT OFFICE

2,101,816

## GALVANIZING COMPOSITION

Frank D. McBride, Philadelphia, Pa.

No Drawing. Application January 21, 1937,  
Serial No. 121,593

3 Claims. (Cl. 148—24)

This invention relates to a galvanizing composition.

Heretofore in the use of galvanized materials the galvanizing has become damaged in one way or another as, for example, by wear or in the process of welding, fabricating, assembly, or otherwise.

The repair of damaged galvanizing has been attempted with the use of a tin-lead solder, but such has proved unsatisfactory, more especially because such a solder offers no protection from rust and corrosion. Again, repair has been attempted with the use of zinc, alone or with a flux, but such has proved unsatisfactory since it is impossible to secure a perfect amalgamation of the zinc with the base metal and the temperature necessarily used for application of the zinc, due to the high melting point, causes the galvanizing surrounding the point of repair to be burned and oxidized.

Now in accordance with this invention, a galvanizing composition is provided with which the repair of worn or damaged galvanizing may be readily accomplished. More particularly, with use of the composition according to this invention a zinc coating, fused with and affording the base metal protection equal to that of the original galvanizing surrounding a damaged or worn portion, may readily be obtained; and with use of a low temperature precluding the burning of or other damage to the surrounding galvanizing.

The composition in accordance with this invention comprises an alloy including lead, tin and zinc or cadmium or a mixture thereof, admixed with a flux.

In the composition according to this invention, zinc and cadmium will be full equivalents one for the other and it will be understood that hereafter and in the claims appended hereto where the term "zinc" is used, cadmium is contemplated as the equivalent.

Generally speaking, zinc or cadmium, or a mixture thereof, will be included in the alloy desirably in amount of from about 40% to about 50%. Where both zinc and cadmium are included, they may be included in any proportion to each other, but desirably will be in the proportion of about 1-75 parts of cadmium to about 99-25 parts of zinc.

Lead and tin will be included in the alloy primarily to reduce the melting point thereof. The amount of lead and tin taken together will be included in amount of from about 50% to about 60%. The proportion of lead to tin may vary,

but desirably they will be included in the proportion of about 70%-30% of tin.

The flux will comprise any suitable flux having the property of dissolving metal oxide in a dry state, for example, triethanolamine, aniline hydrochloride, zinc chloride, ammonium chloride, a mixture of zinc chloride and ammonium chloride in the proportion, for example of 60% zinc chloride and 40% ammonium chloride, etc. Desirably the flux will include a preserver, as magnesium carbonate or equivalent, in amount of from about 1% to about 3%, to negative hardening of the composition from chemical action.

The composition will include the metallic ingredients or alloy and the flux in proportion with the range 30% metal—70% flux to 70% metal—30% flux.

In preparing the composition, the metallic ingredients will be alloyed, the alloy, desirably, powdered or granulated and then mixed with the flux.

In using the composition for the repair of worn or damaged galvanizing, it may be applied to the work in powdered or granulated form, as with a blow torch, at a temperature of, for example, 500-600° F.

More specifically, a desirable composition in accordance with this invention, which will be readily applied without preparation, as by cleaning, of the base metal and which will effectively combine with the base metal and surrounding galvanizing and afford protection to the base equal to that of hot-dipped galvanizing, will comprise an alloy of 50% zinc, 15% lead and 35% tin admixed in powdered form with a flux in the proportion of 65% alloy and 35% flux.

In using the composition according to this invention for the repair of worn galvanizing, or for the replacement of galvanizing which has been burnt off in welding, it will be found that an efficient coating of galvanizing, fused or amalgamated with the base metal and with the galvanizing surrounding the worn or damaged portion will be obtained and the coating will afford efficient protection from rust and corrosion.

The composition according to this invention permits repairs to galvanizing to be made at any point and on parts of structures where in fabrication or assembly damage to galvanizing has occurred and unless the work be exceptionally dirty no preparation of the surface will be necessary.

What I claim and desire to protect by Letters Patent is:

1. A galvanizing composition comprising an alloy of lead, tin and zinc in which the zinc is

present in amount not less than 40% of the alloy, the lead and tin forming the balance of the alloy, and a flux capable of dissolving metal oxide in a dry state admixed with the alloy.

5 2. A galvanizing composition comprising an alloy of lead, tin and zinc in which the zinc is present in amount within the range 40%-50% of the alloy, the lead and tin forming the balance of the alloy, and a flux capable of dissolving metal oxide in a dry state, the flux and alloy be-

ing in proportion within the range 30% alloy—70% flux to 70% alloy—30% flux and the flux being admixed with the alloy.

3. A galvanizing composition comprising an alloy of lead, tin and zinc in which the zinc is present in amount not less than 40% of the alloy, the lead and tin forming the balance of the alloy, and a flux consisting of 60% zinc chloride and 40% ammonium chloride admixed with the alloy.

FRANK D. McBRIDE. 10